

## UNITED STATES PATENT OFFICE

1,955,678

FUR TREATING COMPOSITION AND  
PROCESSWarren C. Mercier, Danbury, Conn., assignor to  
American Hatters and Furriers Company,  
Danbury, Conn., a corporation of New YorkNo Drawing. Application March 28, 1931,  
Serial No. 526,131

15 Claims. (Cl. 8—21)

This invention relates to the art of treating fur and like fibers to give them felting properties, and to a composition of matter adapted to impart such properties to the fibers.

5 One of the objects of the invention is to provide a composition and process adapted for the manufacture of strongly adhering felt. Another object of the invention is to provide a composition and process which gives fur tight felting qualities. Another object of the invention is to provide a composition and process adapted for the production of a fast-shrinking fur. Another object of the invention is to provide a composition and process adapted to produce a quick 10 starting fur. Another object of the invention is to provide a composition and process that will not discolor the fur fibers.

Another object of the invention is to provide fur or like fibers which may be immediately felted after treatment according to the invention. Another object of the invention is to provide fur or like fibers which do not deteriorate materially over a long period of time. Another object of the invention is to so treat fibers adapted to the 15 production of felt that a low grade of fibers may be used, either as filler or otherwise. Another object of the invention is to achieve a thorough oxidation of a constituent substance of the fibers. Other objects will be in part obvious or in part 20 pointed out hereinafter.

The invention accordingly consists in the features of composition, combinations of elements, and in the several steps and relation and order of each of said steps to one or more of the others 25 thereof, all as will be illustratively described herein, and the scope of the application of which will be indicated in the following claims.

As conducive to a readier and clearer understanding of the several features, it may be noted 30 that the subject matter of this invention deals primarily with a composition of matter adapted to affect or modify fur or similar fibrous animal products in order that felt may be manufactured therefrom into such articles as hats, and also 35 with the art of treating such fibers to give them felting qualities. A process that imparts felting qualities to fibers is known in the art as carrottting. The felting of such fibers involves the shrinking of the body which they collectively 40 compose and a thickening of the fibers in the sense that the finished, felted product contains a greater number of them to the square inch and the body which they compose is usually actually thicker in measurement at the completion of the 45 felting operation than it was when initially

formed. Considering, by way of example, the manufacture of a hat, the treated fibers are deposited loosely upon a cone, and, after being wet, are removed from the cone and are found to cling together and form a definite object 50 which has certain dimensions. As a result of the felting of these fibers, by the subsequent operations known as starting and sizing, the length and breadth of the hat body are greatly reduced, while the material as a whole gains in thickness 55 and strength. Considering the individual fibers, this felting operation involves a relative movement among them whereby, being initially spread out quite thinly, they are finally, at the completion of the operation, densely and tightly compacted together and intertwined, giving the resultant hat adequate strength to withstand ordinary usage.

The exact nature of the change wrought in a fur fiber by any particular carrottting operation, 60 whereby, under the manipulation given to a body during the felting operation it acts to produce, collectively with other fibers, the transformation of the product above indicated, is in dispute, various authorities holding different theories 65 which are not entirely in harmony with each other. Although, not being certain which if any of the already advocated theories is correct, I shall not herein enter into any of them in detail, I may use certain terms which have a significance in connection with one or more of such theories, but I wish it understood that my invention is not limited by any theory, being fully pointed out herein and distinctly claimed so 70 that any one skilled in this art can understand how to practice the invention and will recognize what is reserved to me by the claims.

Irrespective of particular theories of carrottting and felting, it is generally understood that properly carrotteted fur has the property of wetting 75 when immersed in the hot water that is used in the starting and sizing operations, so-called. Ordinary uncarrotteted fibers will not readily wet, and a carrottting operation involves a cleansing or hydrolyzing action which affects or modifies some 80 constituent substance of or on the fiber so as to permit it to wet. A heretofore widely used carrottting agent is mercury nitrate, so called, which chemically speaking is supposed to be mercuric nitrate and nitric acid, and this substance is recognized, when in water solution, as a hydrolyzing agent, being of a corrosive nature with an acid reaction. This heretofore widely used carrott has been known or designated in the art as "mercury carrott" or "mercury nitrate" 85

carrot" and how the solution thereof is made is widely known; its acid reaction or acid content has been well recognized, and, being made by dissolving mercury in nitric acid (as fur cutters 5 almost invariably have made it up), the resultant solution includes mercury nitrate and nitric acid, whence come the "mercury" or "mercury nitrate" designations of the carroting solution and its known or recognized acidity or acid content. Fur 10 carroted with this heretofore widely used and well-known solution or carrot is known to increase in feltability with aging, and it has been assumed that this is because this mercury salt is 15 deliquescent, thus causing the fur so carroted to absorb moisture from the air and causing a continuation of the hydrolyzing or cleansing action. I have found in accordance with certain features of my invention that the use of a strong oxidizing agent with a suitable hydrolyzing agent 20 so assists and accelerates the carroting that fur treated with these agents does not require aging and, as a felting substance, presents marked advantages over fibers not so treated.

The usual method of applying a carroting solution to fur is to brush it into the fur while the latter is still on the skin. In carrying out the process of this invention, I preferably apply the solution of the invention in this manner. The fur is then dried and thereafter may be removed 25 from the skin and immediately made into felt, but if, from business or commercial considerations, it is desirable to hold the fur in stock, it may be kept in storage and will be found to undergo practically no deterioration over a long 30 period. Preferably the solution used is a solution of an acid hydrolyzing agent and a strong oxidizing agent. The hydrolyzing agent may be the above-mentioned acidic hydrolyzing agent derived, as above set forth, by way of the "mercury 35 nitrate" or so-called "mercury" solution, which, as above pointed out, is acid in reaction, containing as it does nitric acid, and includes mercury nitrate as such, and the strong oxidizing agent may be hydrogen peroxide ( $H_2O_2$ ) of in 40 the neighborhood of 20 volumes of the gas to one volume of the liquid, or stronger. Markedly 45 different results are obtained by using hydrogen peroxide of this order of strength over what is possible with weaker hydrogen peroxides.

As I understand it, active qualities of hydrogen peroxide are principally due to the fact that it liberates atomic oxygen, which is nascent oxygen or oxygen in a much more chemically reactive form than the molecular oxygen such as 50 is a constituent part of the atmosphere. The higher the concentration of this atomic oxygen in the hydrogen peroxide solution, the more atomic oxygen will be liberated, and I have found that, with respect to fur fibers, increasing 55 the strength to high concentrations results in a different action upon the fur, possibly due to the breakdown of certain constituent fur substances or molecules, which coat differently or negatively with, or perhaps are able to withstand, an ordinary oxidizing agent, such as 60 represented by hydrogen peroxide in the weaker 65 solutions.

To illustrate further how I employ, in coaction with an acid hydrolyzing agent, a suitable oxidizing agent, I may first note that there is available 70 a so-called 100 volume hydrogen peroxide containing 100 volumes of the oxygen gas to 1 of water, and this substance is known as "Albone C." There is also a still more concentrated hydrogen 75 peroxide containing 200 volumes of oxygen gas to

1 of water. I may use either of these substances as the strong oxidizing agent, and I may dilute either of them with water to obtain the exact desired concentration for a particular kind of fur or other fibers, or to obtain particular qualities 80 in such fibers. Those skilled in this art will understand that owing to variations between the characteristics of different kinds of fur, and owing to different manufacturing conditions and differences of temperature and humidity, it is 85 desirable to have different strengths of solutions for different conditions.

As illustrative embodiments of the composition and process of the invention, I give the following preferred examples of solutions:—

1. To 20 parts, by volume, of "Albone C" which is, as above stated, 100 volume  $H_2O_2$ , add 80 parts, by volume, of water (thus reducing the  $H_2O_2$  to 20 volume strength), and to the solution so obtained add 100 parts, by volume, of 3° Baumé 95 solution of mercury nitrate;

2. To 1 part, by volume, of "Albone C" which is, as above stated, 100 volume  $H_2O_2$ , add 1 part, by volume, of 20° Baumé solution of mercury nitrate;

3. To 1 part, by volume, of 200 volume  $H_2O_2$ , add 1 part, by volume, of 30° Baumé solution of mercury nitrate.

As preferred ranges of strengths of the hydrogen peroxide on the one hand, and of the mercury nitrate when that is used as the hydrolyzing agent on the other hand, the range of the hydrogen peroxide is from 50 to 100 volumes, and the range of the mercury nitrate is from 7° to 15° Baumé. Within these ranges I have achieved 105 very excellent results, using 10 parts by volume of hydrogen peroxide to 1 part by volume of mercury nitrate, and 10 parts by volume of mercury nitrate to 1 part by volume of hydrogen peroxide, and intermediate proportions of these two agents. 110

By "mercury nitrate" I mean and intend the known carroting substance passing by that name, and mercury nitrate, as it is known and understood in the art of carroting fur, is acid in reaction and, I am informed and believe, consists 120 chemically largely of mercuric nitrate— $Hg(NO_3)_2$ —and nitric acid— $H(NO_3)$ . At all events it is and was made by completely dissolving mercury in nitric acid. Of course the substances are in an ionic state, water is present or 125 added, and there may be other substances present. Among the latter I believe some mercury oxide— $HgO$ —to be formed, and acts to a certain extent as an oxidizing agent. The action of the oxygen in this oxygen carrier (which, however, 130 is substantially insoluble and does not release any atomic oxygen) might produce a mild oxidizing action upon the fibers if it is at all available for any such action; at all events, whatever oxidizing action of this heretofore widely used mercury nitrate carrot may be, it is not at all comparable, as I have found in practice, with the character of action or with the results achieved by the solution of my invention. Any oxidizing action of heretofore known carrots is of a different 135 character and order from the strong oxidizing action of the atomic oxygen released by the concentrated solutions of hydrogen peroxide above given as a result of certain coactions that take place with the acid hydrolyzing agent. Certain 140 advantages follow from the use of mercury nitrate as the hydrolyzing agent by reason, among others, of the fact that the acid, besides acting as a hydrolyzing agent on the constituents of the fur fibers, coacts with, and act directly upon, 145

150

the hydrogen peroxide or the atomic oxygen made available by the latter to multiply the oxydizing power thereof. In this connection, it may be noted that a fur fiber is of such a complex nature that different constituent parts of it are affected by different specific agents and different strengths of the same agent. I believe that there is some action, interaction, or joint action among, by or between the several elements, ions, compounds or radicals of my new carroting solution that produces or effects a markedly greater oxidizing of the fur than it has been possible to achieve by any prior carroting solution or process.

Certain marked advantages result from the use of the composition and process herein described. For example, it is possible to make a very tight felt with fur carroted as herein set forth and the fur adheres very strongly, thus making a strong felt. I have found that fur treated according to my invention starts very rapidly, by which is meant that in the so-called starting operation the fibers go together quickly and shrinking proceeds with great rapidity. In fact, fur so treated is found to be a fast-shrinking fur, shrinking rapidly not only during the starting operation but also during the sizing operation. It is understood among those skilled in this art that the shrinking qualities of fur are important from the manufacturing standpoint; a fur which shrinks rapidly may be turned into completed articles more quickly and with less effort on the part of the operatives than fur not having such qualities. Nevertheless, when a piece of felt made of fur treated in accordance with the invention arrives at the size desired, it stops felting and attains a stability. The shrinking and feltable qualities of fur may be plotted against time and it will be found that some furs start slowly and accelerate towards the ends of the process so that it is difficult to hold them at the correct size. The desired property of fur in this respect is to have it start quickly and felt rapidly up to finished size and then definitely attain stability, and fur treated according to the invention has this property.

A very important characteristic of the carroting composition and process of the invention resides in the fact that the use thereof eliminates all discoloration of the fur. White fur carroted according to the invention is still white. The old mercury nitrate process resulted in discoloration of the fur; when artificial heat was used for drying, discoloration was accentuated and the fur was of the color of a carrot (whence the word "carroting"). I am not certain in what manner the hydrogen peroxide acts to prevent discoloration, but at all events the result is marked, and fur treated according to the invention can be successfully dyed into the lighter shades;—something which cannot be achieved with mercury nitrate carroted fur.

Many other advantages inhere in the invention. Fur treated according to the invention may be dried either with or without artificial heat, and may be used immediately after being carroted or at a later time. It is found that a newly formed hat bat of fur treated according to the invention will hold air, thus showing that the fibers started to adhere and shrink immediately they were wet. Also, hat bats or bodies made from fur treated according to my invention, as well as the carroted fur itself, may be stored or carried in stock over substantial periods of time adequate to meet the various needs or conditions met with in the fur-preparing and felt-hat manufacturing arts, without detriment-

tal deterioration and without harmful chemical or other change. Moreover, owing to the fast-shrinking and strongly adhering qualities of this fur, a large amount of per se non-feltable, otherwise known as "filler", fur may be mixed in, and in fact large quantities of fiber other than fur may be mixed with fur treated according to the invention, resulting in a good quality of felt at low cost.

The fur treated according to the invention may be dyed in the usual manner, and it is found that there is no undercast to the fur after dyeing.

From the above it will be readily seen that there is herein provided a composition of matter and an art of preparing fur or similar material which attains the objects of this invention, including many distinct practical and useful advantages. Furthermore, the art of preparing the material is one which may be efficiently carried on in a practical commercial manner.

As various possible embodiments might be made of the above invention, and as many changes might be made in the embodiments above set forth, without departing from the scope of the invention, it is to be understood that all matter hereinbefore set forth is to be interpreted as illustrative and not in a limiting sense.

I claim:

1. A carroting solution comprising an aqueous solution of mercuric nitrate, hydrogen peroxide, and nitric acid.

2. The process of carroting fur which comprises subjecting the fur to the action of an aqueous carroting solution of mercuric nitrate, hydrogen peroxide and nitric acid.

3. As a composition of matter for the carroting of fur and the like, the reaction product of a solution of mercury nitrate, acid in reaction, in combination with atomic oxygen.

4. The process of preparing fur or the like for felting which comprises treating fur fibers with the reaction product of an aqueous solution of mercury nitrate, acid in reaction, and atomic oxygen.

5. The process of preparing fur or the like for felting which comprises treating fur fibers to the action of an aqueous carroting solution of an acid hydrolyzing agent and hydrogen peroxide.

6. As a composition of matter for the carroting of fur and the like, a hydrolyzing and oxidizing carroting solution containing hydrogen peroxide and an acid, the acid having a hydrolyzing action on the material of the fur fibers and coacting with the hydrogen peroxide to multiply the oxidizing action thereof.

7. As a composition of matter for the carroting of fur and the like, a carroting solution comprising the reaction product of a solution of hydrogen peroxide of at least 20-volume strength and a solution of mercury nitrate, acid in reaction, of at least 3° Baumé strength.

8. As a composition of matter for the carroting of fur and the like, a carroting solution comprising the reaction product of a solution of hydrogen peroxide of a strength of 50 volumes or more and a solution of mercury nitrate, acid in reaction, of a strength of 15° Baumé or less.

9. As a composition of matter for the carroting of fur and the like, a carroting solution comprising the reaction product of a solution of hydrogen peroxide of a strength ranging from 50 volumes to 200 volumes and a solution of mer-

80

85

90

95

100

105

110

115

120

125

130

135

140

145

150

- cury nitrate, acid in reaction, ranging from 30° Baumé to 3° Baumé.
10. As a composition of matter for the carrott-  
ing of fur and the like, a carrott-  
ing solution com-  
prising the reaction product of a solution of  
hydrogen peroxide of a strength in the neigh-  
borhood of 100 volumes and a solution of mer-  
cury nitrate, acid in reaction, of a strength sub-  
stantially in the range of 7° to 15° Baumé.
- 10 11. As a composition of matter for the carrott-  
ing of fur and the like, the reaction product of a  
solution of mercury nitrate, acid in reaction, of a  
strength between 30° Baumé and 3° Baumé, in  
combination with atomic oxygen.
- 15 12. The process of preparing fur or the like  
for felting which comprises treating fur fibers to  
the carrott-  
ing action of the reaction product of a  
solution of an acid fur-hydrolyzing agent and a  
solution, of a strength of 50 volumes or more, of  
20 hydrogen peroxide.
13. The process of preparing fur or the like  
for felting which comprises uniting hydrogen  
peroxide with an agent which multiplies the oxi-  
dizing power of the hydrogen peroxide and which  
is also an acid fur-hydrolyzing agent, and then  
subjecting the fur fibers to the multiplied oxi-  
dizing action of the hydrogen peroxide and to the  
hydrolyzing action of the acid hydrolyzing agent.
14. The process of preparing fur or the like for  
felting which comprises subjecting a solution of  
an agent which normally is capable of providing  
atomic oxygen for oxidation to the action of an  
oxidizing-power-multiplying agent which is also  
an acid fur-hydrolyzing agent, and subjecting the  
fur fibers to the multiplied oxidizing action of said  
first-mentioned agent and to the hydrolyzing  
action of said second-mentioned agent.
15. The process of preparing fur or the like for  
felting which comprises subjecting the fur fibers  
to the action of a carrott-  
ing solution of an acid  
agent for hydrolyzing constituents of the fur  
fibers and atomic oxygen for oxidizing con-  
stituents of the fur fibers.
- 90 95  
WARREN C. MERCIER.
- 25 100
- 30 105
- 35 110
- 40 115
- 45 120
- 50 125
- 55 130
- 60 135
- 65 140
- 70 145
- 75 150